

## UNITED STATES PATENT OFFICE

2,373,286

## MINERAL OIL COMPOSITION AND IMPROVING AGENT THEREFOR

Darwin E. Badertscher, Robert H. Williams, and Henry G. Berger, Woodbury, N. J., assignors to Socony-Vacuum Oil Company, Incorporated, New York, N. Y., a corporation of New York

No Drawing. Original application October 5, 1939, Serial No. 298,052, now Patent No. 2,279,218, dated April 7, 1942. Divided and this application January 8, 1942, Serial No. 426,002

6 Claims. (Cl. 252—54)

This application, which is a division of our copending application Serial No. 298,052, filed October 5, 1939, now Patent No. 2,279,218, issued April 7, 1942, relates to viscous mineral oil compositions of the lubricant and dielectric types which have been improved in one or more of their various properties by having admixed therewith a minor proportion of mineral oil-improving agent. More specifically, the invention is concerned with the production of a novel class of mineral oil-improving agents and with the production of improved mineral oil compositions of the viscous type containing one or more of these novel improving agents.

It is well known to those familiar with the art that the deteriorating effect of oxidation and continued use upon a mineral oil fraction manifests itself in various ways, depending upon the source of the oil—that is, the crude from which it is derived—the refining treatment to which the oil has been subjected, and the particular conditions under which the oil is subjected to oxidation. Motor oils, for example, especially those refined by certain solvent-extraction methods, tend to oxidize when subjected to high temperatures and form products that are corrosive to metal bearings. This corrosive action may be severe with certain bearing metals such as the hard metal alloys of the cadmium-silver and copper-lead types, and the class of improving agents contemplated herein are particularly useful as inhibitors of oxidation and the attending bearing-corrosion in oils of this character.

The oil-improving agents contemplated herein also find valuable application in the field of motor-lubrication as inhibitors of the formation of materials which lead, on accumulation, to the sticking of piston rings and the filling of the slots in oil rings.

Certain of these improving agents are also useful in oils which have been refined for turbine or transformer use, particularly those which have been highly refined to retard the deterioration of such oils and the attending development of acid or sludge which takes place under the conditions of use.

Although the general class of compounds or reaction products contemplated herein finds application principally in the field of oxidation-inhibitors, and particularly as improving agents for internal combustion engine lubricants, it is to be understood that these improving agents may effect improvement in other respects or properties, such as load-carrying capacity, and, as indicated above, certain members of the class, at least, are effective acid-inhibitors for highly refined turbine and transformer oils. In this same connection our invention contemplates, as an especially preferred group or type of improving agents falling within the general class, com-

5 pounds or reaction products which are multifunctional in that they possess in addition to the inhibiting properties mentioned above, the property of improving the pour point of the oil to which they are added.

10 The oil-improving agents contemplated herein have as their characterizing constituent a reaction product obtained by reacting a phosphorus pentachloride with an aromatic hydroxycarboxylic acid which we may represent by the general formulae:



and



25

wherein the R's represent radicals selected from the group consisting of hydrogen, alkyl, aryl, 30 aralkyl, and alkaryl radicals. The foregoing reaction may be represented by the following equation, wherein the ortho-hydroxy acid is used for purposes of illustration:



Because of uncertainty as to the molecular structure of this reaction product we prefer to identify it by its empirical formula C<sub>7</sub>H<sub>4</sub>O<sub>3</sub>Cl<sub>3</sub>P or merely as a reaction product instead of indulging in speculation as to the structural formula. It will be observed that in the foregoing illustrative equation and reaction the aromatic hydroxycarboxylic acid used was an unsubstituted 50 ortho-hydroxybenzoic acid (salicylic acid); and while the ortho-hydroxybenzoic acid (both substituted and unsubstituted) and phosphorus pentachloride are considered preferred reactants for obtaining this group of compounds, it is to be understood that this invention includes mono-

and poly-cyclic aromatic hydroxycarboxylic acids in general and phosphorus pentahalides as reactants for obtaining this particular group of reaction products which are effective oil-improving agents.

As an example of a substituted ortho-hydroxybenzoic acid which may be reacted with a phosphorus pentahalide, we may mention thymotinic acid (methyl isopropyl salicyclic acid) having the general formula:



These two acids, salicyclic acid and thymotinic acid, will be used herein to illustrate the manner of synthesizing the various oil-improving agents and to demonstrate their effectiveness in mineral oil compositions.

#### EXAMPLE

##### SYNTHESIS OF $\text{PCl}_5$ -AROMATIC ORTHO-HYDROXY CARBOXYLIC ACID REACTION PRODUCTS

###### (a) $\text{PCl}_5$ -salicyclic acid reaction product

One mol of salicyclic acid and one mol of phosphorus pentachloride were mixed together in a large flask fitted with a stirrer and reflux condenser. The mixture was heated on a water bath to a temperature not exceeding 80° F. and stirred until HCl evolution ceased. Hydrogen chloride evolution commenced when the reactants were mixed and became quite vigorous at the elevated temperature. The resulting product was a light-colored liquid which will be hereinafter referred to as the "Salicyclic- $\text{PCl}_5$  product."

###### (b) $\text{PCl}_5$ -thymotinic acid reaction product

Following the same procedure described above, equal molecular proportions of thymotinic acid and phosphorus pentachloride were reacted together to yield a brown liquid product which will be hereinafter referred to as "Thymotinic- $\text{PCl}_5$  product."

###### (c) $\text{PCl}_5$ -beta-hydroxy-alpha-naphthoic acid reaction product

Fifteen grams of beta-hydroxy-alpha-naphthoic acid and 22½ grams of  $\text{PCl}_5$  were stirred together without external application of heat. A spontaneous reaction occurred, accompanied by a temperature rise from 28° C. to 42° C., forming a dark oil. This was taken up in 100 c. c. of petroleum ether and 10 c. c. of benzene and filtered. The solvents were partially removed in a vacuum dessicator, yielding a white crystalline solid with a melting point slightly above room temperature. This product will be identified herein as "Hydroxy-naphthoic- $\text{PCl}_5$  product."

As was pointed out above, the compounds or reaction products contemplated herein are effective to inhibit the corrosive action of mineral oil fractions, such as solvent-refined oil, normally corrosive to hard metal alloy bearing metals typified by cadmium-silver and copper-lead alloys. In this same regard, our invention contemplates, in addition to mineral oil fractions containing the improving agents contemplated herein, a method for lubricating alloy bearings which involves the use of a lubricant containing one or

more of these improving agents to provide the lubricant film.

To demonstrate the effectiveness of the improving agents contemplated herein as inhibitors of corrosive action of the type above referred to, samples of a motor lubricating oil and of an oil blend containing a representative improving agent, "Salicyclic- $\text{PCl}_5$  product," were tested by suspending a 6-gram section of a hard metal alloy bearing in a 30-gram sample of the oil or blend and heating it to about 175° C. for 22 hours while bubbling a stream of air against the surface of the bearing. The weight loss in milligrams of the bearing section is interpreted as a measure of the corrosiveness of the oil. The alloy bearing section in both cases was from a cadmium-silver bearing, and the oil was a commercial S. A. E. 20 solvent-refined motor oil. Results of this test are given below in Table I.

TABLE I

|    | Improving agent                    | Weight percent in oil | Weight loss in milligrams |
|----|------------------------------------|-----------------------|---------------------------|
| 25 | None                               |                       | 35                        |
|    | Salicyclic- $\text{PCl}_5$ product | 0.25                  | 1                         |

To further demonstrate the effectiveness of the improving agents contemplated herein as inhibitors of corrosive action of the type referred to above, samples of a motor lubricating oil and of an oil blend containing the same representative improving agent, "Salicyclic- $\text{PCl}_5$  product," were subjected to the Lauson engine test. These tests were made with a conventional single-cylinder, 4-cycle, liquid-cooled Lauson engine which had been equipped with an electrically heated sump, an oil pump, and a reflux condenser attached to the cooling jacket. During the test operation the temperature of the oil going into the engine from the sump was maintained at 300° F., and it was circulated at the rate of 40 gallons per hour. The temperature of the cooling jacket was about 212° F., and the engine was operated at a speed of approximately 1810 R. P. M., the power output at this speed (about 0.5 H. P.) being absorbed by an A. C. induction motor coupled directly to the crank shaft of the engine. The oil, or oil blend, under test was inspected at the end of 12 hours, and again at the end of 24 hours, and finally at the end of 36 hours when the test run was completed. At each inspection (12, 24, and 36 hours) the oil, or oil blend, was tested for acidity or neutralization number (N. N.) and Kinematic viscosity (K. V.) at 210° F. At the 24 hour and 36 hour inspections, the oil, or oil blend, was tested still further for the amount of A. S. T. M. naphtha insolubles. The mineral oil stock used in these tests was an S. A. E. 10 solvent-refined motor oil. The results obtained are listed in Table II below.

TABLE II

| Improving agent                    | Weight percent in oil | N. N. |     |     | K. V. @ 210° F. |      |       | A. T. S. M. naphtha insolubles |      |      |
|------------------------------------|-----------------------|-------|-----|-----|-----------------|------|-------|--------------------------------|------|------|
|                                    |                       | 12    | 24  | 36  | 12              | 24   | 36    | 12                             | 24   | 36   |
| None                               |                       | 1.5   | 5.6 | 9.2 | 6.11            | 7.51 | 10.51 | 0.23                           | 0.23 | 0.92 |
| Salicyclic- $\text{PCl}_5$ product |                       | 1.0   | 0.5 | 0.5 | 0.6             | 5.67 | 5.75  | 5.85                           | 0.09 | 0.12 |

In addition to the foregoing motor oil tests, a typical improving agent contemplated herein was blended with a motor oil and subjected to an ac-

celerated engine operation test to evaluate its ability to prevent ring-sticking, etc., in engine operation. The engine employed in the test was a standard C. F. R. "knock test" engine and the test involved operating the engine first with the oil and then with the oil blend at an approximate speed of 1,200 R. P. M. with the throttle set just below detonation, using a compression ratio of 7:1 and a jacket temperature of 400° F.

At the end of 28-hour test runs, the following inspections were made:

I. The piston:

- (a) Degree of ring-sticking (0° being an entirely free ring and 360° a totally stuck ring)
- (b) Per cent of filling of oil slots
- (c) Deposits (grams)

II. Used oil:

- (a) Kinematic viscosity (K. V.) at 210° F.
- (b) Neutralization number (N. N.)

The results obtained are listed in Table III below, where "oil A" is the motor oil blank and "oil B" is the same oil containing 1.0% of the "Salicylic-PCl<sub>5</sub> product."

TABLE III

| Oil | Degrees stuck |     |     |     |     | Slots, per cent filled |    |    | Total deposits | Used oils     |       |
|-----|---------------|-----|-----|-----|-----|------------------------|----|----|----------------|---------------|-------|
|     | 1             | 2   | 3   | 4   | 5   | 3                      | 4  | 5  |                | 210° F. K. V. | N. N. |
| A   | 360           | 360 | 360 | 360 | 360 | 70                     | 70 | 90 | 13.9           | 30.02         | 2.2   |
| B   | 0             | 0   | 0   | 0   | 0   | 10                     | 20 | 5  | 7.2            | 26.34         | 1.6   |

The ability of the improving agents contemplated herein to increase the load-carrying capacity of lubricants has been demonstrated with the "Salicylic-PCl<sub>5</sub> product." A typical gear oil which failed in the Almen test at a load of 3,000 pounds passed the same test at a load of 30,000+ pounds when blended with 5.0% of the "Salicylic-PCl<sub>5</sub> product."

The amount of improving agents which may be used in the oil will vary more or less with the oil and the conditions of use, but in general the desired improvement can be effected with amounts ranging from about 0.01% to about 10%.

It is to be understood that while we have herein described certain preferred procedures for synthesizing improving agents of the type contemplated by this invention and have designated certain illustrative reactants which may be employed, the invention is not confined to the specific detailed procedural operations or reactants described but includes within its scope whatever changes fairly come within the spirit of the appended claims.

We claim:

1. An improved mineral oil composition comprising a viscous mineral oil fraction and in admixture therewith a minor proportion of a reaction product obtained by reacting a phosphorus pentachloride with an aromatic hydroxycarboxylic acid, said mineral oil composition being free of sulfur.

2. An improved mineral oil composition comprising a viscous mineral oil fraction and in admixture therewith a minor proportion of a reaction product obtained by reacting phosphorus pentachloride with an ortho-hydroxybenzoic acid, said mineral oil composition being free of sulfur.

3. An improved mineral oil composition comprising a viscous mineral oil fraction and in ad-

mixture therewith a minor proportion of a reaction product obtained by reacting phosphorus pentachloride with salicylic acid, said mineral oil composition being free of sulfur.

5. An improved mineral oil composition comprising a viscous mineral oil fraction and in admixture therewith a minor proportion of a reaction product obtained by reacting phosphorus pentachloride with thymotinic acid, said mineral oil composition being free of sulfur.

10. An improved mineral oil composition comprising a viscous mineral oil fraction and in admixture therewith a minor proportion of a reaction product obtained by reacting phosphorus pentachloride with a compound selected from the group having the general formulae:



25 and



35 in which the R's represent radicals selected from the group consisting of: hydrogen, alkyl, aryl, aralkyl, and alkaryl radicals, said mineral oil composition being free of sulfur.

6. The method of lubricating relatively moving metallic bearing surfaces having the corrosion-susceptibility of hard metal alloys of the cadmium-silver type which comprises maintaining between the bearing surfaces a lubricant film having as a primary lubricating constituent the combination of a major portion of a mineral oil normally corrosive to alloys of the cadmium-silver type and a minor proportion of a reaction product obtained by reacting phosphorus pentachloride with a compound selected from the group having the general formulae:



55 and



60 in which the R's represent radicals selected from the group consisting of: hydrogen, alkyl, aryl, aralkyl, and alkaryl radicals, said lubricant film being free of sulfur.

DARWIN E. BADERTSCHER,  
ROBERT H. WILLIAMS,  
HENRY G. BERGER.